

# United States Patent Office

3,184,412

Patented May 18, 1965

1

3,184,412

3,184,412

**LUBRICANTS INHIBITED AGAINST OXIDATION**

Warren Lowe, Berkeley, and Frank A. Stuart, Orinda, Calif., assignors to California Research Corporation, San Francisco, Calif., a corporation of Delaware

No Drawing. Filed Sept. 28, 1962, Ser. No. 227,037  
4 Claims. (Cl. 252—46.7)

This invention pertains to lubricating oil compositions having incorporated therein metal-free detergents. These particular detergents are also effective as oxidation inhibitors.

Present day internal combustion engines operate at high speeds and high compression ratios. When used in the so-called city stop-and-go driving, which includes the greater part of the driving conditions for a large percentage of today's automobiles, the internal combustion engines do not reach the most efficient operating temperature. Under city driving conditions, large amounts of partial oxidation products are formed, and reach the crankcase of the engine by blowing past the piston rings. Most of the partial oxidation products are oil-insoluble, tending to form deposits on the various operating parts of the engine, such as the pistons, piston rings, etc. For the purpose of preventing the deposition of these products on the various engine parts, it is necessary to incorporate detergents in the lubricating oil compositions, thus keeping these polymeric products dispersed in a condition unfavorable for deposition on metals.

For the most part, the detergents which are added to crankcase oils to reduce this formation of sludges and varnishes are metal organic compounds, particularly those compounds wherein the metal is linked to an organic group through an oxygen atom. Although these metal-containing organic compounds have some effectiveness as detergents for dispersing the precursors of the deposits within the oil itself rather than permitting them to form as deposits on the engine parts, they have the disadvantage of forming ash deposits in the engine. These ash deposits lower engine performance by fouling spark plugs and valves, and contributing to pre-ignition.

It is a particular object of this invention to provide lubricating oil composition having incorporated therein metal-free detergents which are also effective as oxidation inhibitors. Thus, these new additives inhibit the oxidation of lubricating oil compositions and also disperse the undesirable polymeric products which are formed.

Therefore, in accordance with this invention, it has been found that lubricating oil compositions particularly useful for heavy duty service are obtained by incorporating therein a product obtained by reacting an alkenyl succinic anhydride and a piperazine derivative, followed by reaction with a dihydrocarbyl dithiophosphoric acid to form a salt thereof.

By the use of lubricating oil compositions containing the salts described herein, diesel and gasoline engine products remain remarkably free of deposits and varnish even under severe operating conditions.

The alkenyl succinic anhydrides which are reactants herein are of the formula

2

n-hexadecenyl, propylene tetramer, butylene trimer, polypropylene polymers containing from 50 to 200 carbon atoms, and polymers of mixtures of 1-butene and isobutene having from 50 to 200 carbon atoms.

5 The piperazine derivatives, which contribute the imide and the basic nitrogen atoms of the reaction products herein, are represented by the formula



15 wherein the  $R^2$  represents a divalent alkylene radical having from 1 to 3 carbon atoms, and  $R^3$  is hydrogen or an alkyl radical having 1 to 3 carbon atoms.  $R^2$  is exemplified by the methylene radical, the ethylene radical, and the propylene radical.  $R^3$  is exemplified by hydrogen, the methyl radical, the ethyl radical, the n-propyl radical, the isopropyl radical, etc.

The dihydrocarbyl dithiophosphoric acids which are used in the salt formation herein are represented by the formula



wherein R<sup>4</sup> and R<sup>5</sup> represent hydrocarbon radicals each having from 1 to 25 carbon atoms, preferably from 4 to 20 carbon atoms. The R<sup>4</sup> and R<sup>5</sup> combined can have a total of from 6 to 50 carbon atoms, preferably from 10 to 40 carbon atoms.

The  $R^4$  and  $R^5$  radicals are exemplified as follows: methyl, ethyl, propyl, isopropyl, etc.

35 Examples of dihydrocarbyl dithiophosphoric acid include dimethyldithiophosphoric acid, methylethyldithiophosphoric acid, diethyldithiophosphoric acid, di-n-propyl dithiophosphoric acid, di-isopropyl dithiophosphoric acid, di-n-butyl dithiophosphoric acid, diisobutyl dithiophosphoric acid, n-butyl-n-amyl dithiophosphoric acid, di-sec-amyl dithiophosphoric acid, methyl-n-hexyl dithiophosphoric acid, isobutyl-n-hexyl dithiophosphoric acid, di-n-octyl dithiophosphoric acid, methylcyclohexyl dithiophosphoric acid, methylcyclohexyl dithiophosphoric acid, di-cyclohexyl dithiophosphoric acid, methylphenyl dithiophosphoric acid, diphenyl dithiophosphoric acid, di-(amylphenyl) dithiophosphoric acid, di-(hexadecylphenyl) dithiophosphoric acid, etc.

The reaction between a piperazine derivative and an alkenyl succinic anhydride can proceed at temperatures ranging from 220° F. to 500° F., preferably from 220° F. to 350° F.

The mol ratio of piperazine derivatives to succinic anhydride can vary from 0.5:1 to 1:1. Preferably, the 55 polyamine-anhydride mol ratio is 0.95:1.

For purposes of simplicity, the product obtained by the reaction of the piperazine derivative and an alkenyl succinic anhydride will be termed a "succinimide."

The succinimides herein are reacted with a dihydro-  
60 carbyl dithiophosphoric acid at temperatures insufficient  
for hydrogen sulfide formation; such temperatures being  
from 50° E. to 220° E. preferably 150° E. to 200° E.

The mol ratio of the succinimide to the dihydrocarbonyl dithiophosphoric acid can vary from 1:1 to 1:4. Preferably, the mol ratio is 1:1.

As identified herein, the term "salt" means the product obtained by reacting the above-identified succinimide with the described dihydrocarboxylic diacid anhydride.

Lubricating oils which can be used as base oils include a wide variety of lubricating oils, such as naphthenic base, paraffin base, and mixed base lubricating oils, other hydrocarbon lubricants, e.g., Lubricating oils containing the described dianhydrocaryl dithiophosphoric acid.



wherein R is a hydrocarbon radical having from 10 to 200 carbon atoms therein, preferably 50 to 200 carbon atoms. Examples of alkenyl radicals include n-decanyl,

rived from coal products, and synthetic oils, e.g., alkylene polymers (such as polymers of propylene, butylene, etc., and the mixtures thereof), alkylene oxide-type polymers (e.g., propylene oxide polymers) and derivatives, including alkylene oxide polymers prepared by polymerizing the alkylene oxide in the presence of water or alcohols, e.g., ethyl alcohol, dicarboxylic acid esters (such as those which are prepared by esterifying such dicarboxylic acids as adipic acid, azelaic acid, suberic acid, sebacic acid, alkanol succinic acid, fumaric acid, maleic acid, etc., with alcohols such as butyl alcohol, hexyl alcohol, 2-ethylhexyl alcohol, dodecyl alcohol, etc.), liquid esters of acids of phosphorus, alkyl benzenes (e.g., mono-alkyl benzene) such as dodecyl benzene, tetradecyl benzene, etc., and dialkyl benzenes (e.g., n-nonyl 2-ethyl hexyl benzene); polyphenyls (e.g., biphenyls and terphenyls), alkyl biphenyl ethers, compounds of silicon (e.g., tetraethyl silicate, tetraisopropyl silicates, tetra(4-methyl-2-tetraethyl) silicate, hexyl(4-methyl-2-pentoxy) disiloxane, poly(methyl) siloxane, poly(methylphenyl) siloxane, etc. Synthetic oils of the alkylene oxide-type polymers which may be used include those exemplified by the alkylene oxide polymers.

The above base oils may be used individually or in combinations thereof, wherever miscible or wherever made so by the use of mutual solvents.

The succinimide-dithiophosphoric acid salt can be used in oils of lubricating viscosity in amounts of 0.10% to 40%, by weight, preferably 0.1% to 15%, by weight, more preferably 1% to 10%.

Thus, the lubricating oil compositions herein contain products obtained by (1) reacting a piperazine derivative with an alkenyl succinic anhydride, followed by (2) reacting the product of (1) with a hydrocarbyl dithiophosphoric acid.

The reaction of an alkenyl succinimide with a piperazine derivative is illustrated in the following example.

#### EXAMPLE I

##### Reaction product of *N*-ethylpiperazine and polybutenyl succinic anhydride

A mixture of 18 grams (0.14 mol) of *N*-( $\beta$ -aminoethyl) piperazine and 200 grams (0.127 mol) of a polybutenyl succinic anhydride wherein the polybutenyl radical was derived from a polyisobutene having about 66 carbon atoms, was blended with agitation at 125° F. in a nitrogen atmosphere. The temperature was increased to 500° F. during a period of one hour, after which the absolute pressure was reduced to about 200 mm. Hg during a period of 30 minutes to facilitate the removal of water and unreacted piperazine. The reaction mixture was then allowed to reach room temperature at this reduced pressure. The reaction product contained 2.59% by weight of nitrogen.

Example II illustrates the reaction of a succinimide and a dithiophosphoric acid.

#### EXAMPLE II

##### Reaction product of a polybutenyl succinimide of $\beta$ -aminoethyl piperazine and a dialkylphenyl dithiophosphoric acid

A mixture of 1140 grams (0.5 mol) of a lubricating oil solution of a polybutenyl succinimide of 2-aminoethyl piperazine and 510 grams (0.5 mol) of a lubricating oil solution of a di(alkylphenyl) dithiophosphoric acid was vigorously stirred on a steam plate for two hours at 180° F. to 200° F., wherein said alkyl radical was a propylene polymer containing 12 to 14 carbon atoms.

Table I presents data obtained with lubricating oil compositions in the L-38 Strip Corrosion Tests, using lead strips. The numbers represent the weight loss in milligrams.

The increase in viscosity figures represent the percent-

age increase in viscosity at 100° F. in the oxidation stability test wherein the oil is heated at 340° F. for 20 hours.

The base oil was a Mid-Continent SAE 30 base oil.

Additive A was a succinimide prepared as in Example I hereinabove.

Additive B was the salt obtained by reacting 1 mol of the succinimide with 1 mol of an alkylphenyl dithiophosphoric acid, wherein the alkyl radical was derived from a propylene polymer having an average of from 12 to 14 carbon atoms.

Additive C was the salt obtained by reacting 1 mol of the succinimide with 1 mol of a dialkyl dithiophosphoric acid, wherein one of the alkyl radicals contained 4 carbon atoms, and the second alkyl radical contained 6 carbon atoms.

TABLE I

| Composition                             | L-38 test result weight loss (mgnms.) | Viscosity increase, percent |
|-----------------------------------------|---------------------------------------|-----------------------------|
| 1. Base oil plus 2.1% weight additive A | 1,747                                 | 640                         |
| 2. Base oil plus 3.1% weight additive B | 22                                    | 11                          |
| 3. Base oil plus 3.1% weight additive C | 20                                    | 3                           |

We claim:

1. A lubricating oil composition comprising a major proportion of an oil of lubricating viscosity and from 0.1% to 40% by weight of a product obtained by (1) reacting an alkenyl succinic anhydride having from 50 to 200 carbon atoms in the alkenyl radical with a piperazine derivative of the formula



wherein  $\text{R}^2$  is a divalent radical having from 1 to 3 carbon atoms and  $\text{R}^3$  is selected from the group consisting of hydrogen and alkyl radicals having from 1 to 3 carbon atoms, wherein the piperazine-anhydride mol ratio is from 0.5:1 to 1:1, followed by (2) reacting the product of (1) with a dihydrocarbyl dithiophosphoric acid of the formula



wherein  $\text{R}^4$  and  $\text{R}^5$  are hydrocarbon radicals each having from 4 to 20 carbon atoms and having a combined number of carbon atoms from 10 to 40, wherein the mol ratio of the product of (1) to dithiophosphoric acid is from 1:1 to 1:4, said reaction (1) being carried out by heating at a temperature from about 220° F. to about 500° F., and said reaction (2) being carried out by heating at a temperature from about 150° F. to about 200° F.

2. A lubricating oil composition according to claim 1 in which the dihydrocarbyl dithiophosphoric acid is alkylphenyl dithiophosphoric acid.

3. A lubricating oil composition according to claim 1 in which the dihydrocarbyl dithiophosphoric acid is dialkyl dithiophosphoric acid.

4. A lubricating oil composition comprising a major proportion of an oil of lubricating viscosity and from 0.1% to 40% by weight of a product obtained by (1) reacting an alkenyl succinic anhydride having from 50 to 200 carbon atoms in the alkenyl radical with *N*-( $\beta$ -aminoethyl piperazine), wherein the piperazine-anhydride mole ratio is from 0.5:1 to 1:1, followed by (2) reacting the

product of (1) with a dihydrocarbyl dithiophosphoric acid of the formula



wherein  $\text{R}^4$  and  $\text{R}^5$  are hydrocarbon radicals each having from 4 to 20 carbon atoms and having a combined number of carbon atoms from 10 to 40, wherein the mole ratio of the product of (1) to dithiophosphoric acid is from 1:1 to 1:4, said reaction (1) being carried out by heating at a temperature from about 220° F. to about 500° F. and said reaction (2) being carried out by heating at a temperature from about 150° F. to about 200° F.

10

15

## References Cited by the Examiner

## UNITED STATES PATENTS

|             |       |                       |           |
|-------------|-------|-----------------------|-----------|
| 2,809,934   | 10/57 | Alford et al. -----   | 252—32.7  |
| 2,973,323   | 2/61  | Millikan et al. ----- | 252—32.7  |
| 5 2,995,568 | 8/61  | Malz et al. -----     | 260—326.5 |
| 3,018,247   | 1/62  | Anderson et al. ----- | 252—32.7  |
| 3,024,237   | 3/62  | Drummond et al. ----- | 252—51.5  |
| 3,058,910   | 10/62 | Culmer -----          | 252—32.7  |
| 3,074,990   | 1/63  | Cyba -----            | 252—32.7  |

DANIEL E. WYMAN, Primary Examiner.

ALPHONSO D. SULLIVAN, Examiner.